# EUROPEAN PATENT SPECIFICATION

(11) **EP 0 374 925 B1**
(45) Date of publication and mention of the grant of the patent: **08.03.1995**
(21) Application number: 89123668.9
(22) Date of filing: 21.12.1989
(51) Int. Cl.: D01F 9/22

(54) **High density graphite fiber and method of manufacture thereof**
Graphitfaser mit hoher Dichte und Verfahren zu deren Herstellung
Fibre de graphite à haute densité et méthode pour sa production

(30) Priority: 22.12.1988 JP 324397/88
(43) Date of publication of application: 27.06.1990
(73) Proprietor: Toho Rayon Co., Ltd., Chuo-ku Tokyo (JP)
(72) Inventor: Ogawa, Hiroyasu c/o Toho Rayon Co., Ltd., Nagaizumi-cho Sunto-gun Shizuoka (JP); Enomoto, Harumitsu c/o Toho Rayon Co., Ltd., Nagaizumi-cho Sunto-gun Shizuoka (JP)
(74) Representative: Hansen, Bernd, Dr. Dipl.-Chem.

(56) References cited:
- EP-A- 0 100 410
- EP-A- 0 159 365
- US-A- 3 454 362

## Description

### FIELD OF THE INVENTION

The present invention relates to a graphite fiber derived from polyacrylic fiber which is useful for reinforcing a composite material, particularly useful for reinforcing a composite material in the aerospace industry. The invention further relates to a method of manufacturing a graphite fiber.

### BACKGROUND OF THE INVENTION

The graphite fibers which have been used in the aerospace industry have a strand tensile modulus of 50x10³ kgf/mm² at the highest and a strand tensile strength of as low as 200 kgf/mm². Accordingly, their use for members in the aerospace industry is limited to a very narrow range. The fibers, even when they are useful, have disadvantages in that they have to be used in a large amount or have to be used in combination with other materials, thus resulting in increased weight.

Such graphite fibers have been made according to the methods disclosed, for example, in U.S. Patent 4,321,446.

Aerospace materials which are repeatedly exposed to high temperatures and low temperatures are required to have high heat conductivity. To meet this requirement, graphite fibers need to have higher density which correlates with the heat conductivity.

Hence graphite fibers are desired to have a high density, a high strength, and a high tensile modulus. Additionally, the graphite fibers are desired to be capable of being used as pseudoisotropic composite material in use for members in the aerospace industry.

Moreover, the graphite fibers are desired to have a small filament diameter. Thus, a graphite fiber has long been desired which is composed of filaments of a small diameter, particularly not more than 7 »m in diameter, and which has a high density, a high strength and a high modulus.

### SUMMARY OF THE INVENTION

An object of the present invention is to provide a graphite fiber which is light in weight and has a high strand tensile modulus and a high strand tensile strength and further which has a high density which contributes to heat conductivity.

Another object of the present invention is to provide a graphite fiber which is suitable for producing a pseudoisotropic composite material.

According to one aspect of the present invention, there is provided graphite fiber derived from an acrylic fiber, which has a fiber density of not less than 1.93 g/cm³, a strand tensile strength of not less than 350 kgf/mm², and a strand tensile modulus of not less than 53x10³ kgf/mm².

According to another aspect of the present invention, there is provided a method for manufacturing a graphite fiber having a fiber density of not less than 1.93 g/cm³, a strand tensile strength of not less than 350 kgf/mm², and a strand tensile modulus of not less than 53x10³ kgf/mm², comprising carbonizing a preoxidized fiber derived from an acrylic fiber and having a fiber density of from 1.32 to 1.40 g/cm³ to obtain a carbon fiber having a nitrogen content of not less than 1.0% by weight based on the carbon fiber weight, a fiber density of not less than 1.79 g/cm³ and an orientation of not less than 79% at a maximum diffraction at 2ϑ=25.3±0.5° in X-ray diffraction angle of the (002) plane of the graphite crystal, and graphitizing the thus-obtained carbon fiber in an inert gas at a temperature of not lower than 2,400°C and under a tension to stretch the fiber at least 3% during the graphitization.

### DETAILED DESCRIPTION OF THE INVENTION

In the present invention the fiber density, the strand tensile strength, and the strand tensile modulus are measured according to JIS R7601, and the diameter of the filament is determined by measuring the sectional area of the filament employing scanning electromicroscopy and converting the obtained value to the true circle diameter.

According to the method of the present invention a graphite fiber having a fiber density of up to about 2.10 g/cm³, a strand tensile strength of up to about 550 kgf/mm², and a strand tensile modulus of up to about 75 x 10³ kgf/mm² can be obtained.

The graphite fiber of the present invention substantially consists of carbon atoms in an amount of 100% by weight. However, nitrogen atoms, oxygen atoms, and hydrogen atoms each may be present in an amount of from 0 to 0.1% by weight, and ash may be present in an amount of from 0 to 0.2% by weight based on the weight of the total weight of the grahite fiber (including such materials, when present).

The ash content is the residue of the graphite fiber after heating the graphite fiber at 650°C in the air for 300 minutes. (The heating is repeatedly conducted until the weight of the residue becomes constant.)
A fiber density of less than 1.93/cm³ leads to decrease in the heat conductivity.

The graphite fiber of the present invention preferably is composed of a filaments of not more than 7 »m in diameter. Although the filament diameter of not more than 7 »m is desirable as mentioned above, an excessively small filament diameter (i.e., less than 0.1 »m), namely extreme fineness thereof, is undesirable because such causes a remarkable increase in fluffing of the strands in ultra-thin sheet materials. A preferred diameter is from 0.5 to 5 »m.

The number of filaments constituting a graphite fiber strand obtained according on the method of the present invention is desirably not overly large, and is preferably from 50 to 15,000 because of the required fineness of the strand. Less than 50 filaments is undesirable since it causes frequent thread breakage rendering difficult the production of thin sheet materials. The filaments constituting the strand are preferably not interlocked but are parallel with each other for producing thinner sheets. The interlocking degree of the filaments in a strand is measured by vertically hanging 300 mm long strand with a load of 0.1 g/d at the lower end thereof, perpendicularly piercing the strand with a chromium plated pin of 1 mm diameter at around the middle of the strand breadth, and measuring the distance that the pin goes down by 10 g of load for 3 minutes. The interlocking degree of the strand is represented by this distance. The interlocking degree is preferably not less than 250 mm.

The graphite fiber of the present invention can be prepared from an acrylic fiber, that is, a polyacrylonitrile fiber or a copolymer fiber composed of preferably about 90% by weight or more, and more preferably about 95% by weight or more, of acrylonitrile, and any vinyl monomers which are copolymerizable with acrylonitrile can be used as the comonomers. For instance, known comonomers can be used, including neutral monomers such as methyl acrylate, methyl methacrylate and vinyl acetate; acrylic acid, methacrylic acid, itaconic acid, maleic acid, vinylsulfonic acid, allylsulfonic acid, methallylsulfonic acid, styrenesulfonic acid and metal salts thereof (such as the sodium salt and potassium salt) and ammonium salts; vinylimidazole, vinylpyrimidine and derivatives thereof; and acrylamide, methacrylamide, etc. The preferred molecular weight of the polymer is about 40,000 to 200,000, more preferably about 60,000 to 150,000 calculated using Staudinger's equation.

The graphite fiber can be obtained by preoxidizing acrylic fiber, carbonizing the thus-obtained preoxidized fiber and the graphitizing the thus-obtained carbon fiber. Methods for producing carbon fiber are known, for example, in U.S. Patents 4,197,279, 4,397,831, 4,347,279, 4,474,906 and 4,522,801, and methods for producing graphite fibers are known, for example in U.S. Patent 4,321,446.

The graphite fiber of the present invention can be obtained by using a specifically selected carbon fiber and by using precisely selected conditions for obtaining the graphite fiber.

The acrylic fiber suitably comprises 50 to 15,000 filaments of a diameter of not more than 13 »m (preferably from 0.1 to 13 »m, more preferably from 0.2 to 10 »m; 0.05 to 1.5d and 0.1 to 1.0d, respectively), having a tensile strength of not less than 3 g/d (preferably of from 3 to 20 g/d, more preferably of from 5 to 15 g/d), a tensile elongation of not less than 5% (preferably from 5 to 15%, more preferably from 7 to 12%), and an orientation degree of not less than 88% (preferably of from 88 to 95%, more preferably of from 90 to 95%) measured at the diffraction angle range of 2ϑ=17.3 ± 0.3° where the maximum diffraction intensity is exhibited in X-ray diffraction. Such an acrylic fiber, can be obtained referring to U.S. Patent Application Serial No. 845,167* The acrylic fiber is preoxidized by heating in air at a temperature below the heat decomposition temperature of the fiber (usually at from 200 to 350°C) under a tension preferably of from 70 to 200 mg/d (more preferably of from 100 to 150 mg/d) for preferably from 5 to 120 minutes (more preferably of from 10 to 60 minutes) to give a fiber density of from 1.32 to 1.40 g/cm³ (preferably from 1.32 to 1.37 g/cm³). Subsequently, the thus obtained preoxidized fiber is carbonized in an inert atmosphere (nitrogen, argon or helium) at a temperature preferably of from 1,100 to 1,430°C (more preferably of from 1,200 to 1,400°C) for preferably from 0.5 to 10 minutes (more preferably from 1 to 5 minutes) under a tension to stretch the fiber (in an extent preferably of from 5 to 20%, more preferably from 8 to 12%) so as to result in a nitrogen content of at least 1.0% (preferably of from 1.0 to 8%, more preferably of from 3 to 5%) by weight in the fiber, an orientation of not less than 79% (preferably of from 79 to 84%, more preferably of from 80 to 84%) measured at a maximum diffraction intensity at 2ϑ=25.3 ± 0.5° (X-ray diffraction angle of the (002) plane of graphite crystal), and a fiber density of at least 1.79 g/cm³ (preferably from 1.79 to 1.85 g/cm³, more preferably from 1.81 to 1.85 g/cm³).
*(corresponding to DE-A1 36 10 517)

Thereafter the thus obtained carbon fiber is stretched at least 3% (preferably from 5 to 15%, more preferably 5 to 10%) during graphitizing in an inert gas atmosphere (argon, helium or nitrogen, preferably argon or helium) at a temperature of 2,400°C or higher (preferably of from 2,400 to 3,300°C, more preferably of from 2,600 to 3,300°C) to produce a graphite fiber. The time period for heating (graphitizing) is usually from about 0.1 to 10 minutes. The graphitization is conducted until the density of the fiber becomes at least 1.93 g/cm³. The thus obtained graphite fiber has an orientation degree (measured as above at 2ϑ=25.3 ± 0.5°), preferably of from 85 to 98%, more preferably from 90 to 98%.

Among the above manufacturing conditions, the fiber density of the preoxidized fiber, the nitrogen content, the orientation degree, the density of the carbon fiber, the graphitization temperature of 2,400°C or higher and the elongation ratio must be met to provide the intended graphite.

By employing the graphite fiber of the present invention in combination with a known resin, unidirectional composite materials, textile composite materials, and pseudoisotropic composite materials by multidirectional lamination can be prepared.

The composite materials reinforced by the graphite fiber of the present invention will enable a weight reduction and thus a speed increase of flying objects, satellites, and space stations etc., in the aerospace field, and similar results with respect to rotating bodies, travelling bodies, etc., in other technical fields.

Examples are shown below together with comparative examples. Unless otherwise mentioned, "%" and "parts" are based on weight in the examples.

### EXAMPLE 1

Various graphite fibers were prepared from an acrylic fiber (filament: 0.5 denier, number of filaments: 6000, tensile strength: 6.8 g/d, tensile elongation: 11%, orientation degree: 90.5% at a diffraction angle of the diffraction peak at 2ϑ=17.3 ± 0.3° in X ray diffraction) composed of 98% of acrylonitrile, 1.5% of methyl acrylate (the molecular weight of the acrylonitrile copolymer was 75,000), and 0.5% of itaconic acid, under the conditions shown in Table 1 regarding the preoxidation treatment (in air, 250°C, tension: 150 mg/d), the carbonization (in nitrogen gas, 3 minutes), and the graphitization (in argon, 3 minutes).

A prepreg containing fiber in an amount of 150 g/m² with a resin content of 37% (based on the weight of the prepreg) was prepared from the thus obtained graphite fiber and a resin component constituted of 50 parts of an epoxy resin: Epikote 828^{®} (made by Yuka Shell Epoxy K.K., bisphenol A diglycidyl ether having an epoxy equivalent of from 184 to 194), 50 parts of Epikote 1002^{®} (made by Yuka Shell Epoxy K.K., bisphenol A diglycidyl ether having an epoxy equivalent of from 600 to 700) and 3 parts of dicyandiamide, by arranging the graphite fiber unidirectionally.

The prepreg was laminated and compression molded at 130°C for 2 hours under a pressure of 7 kgf/cm² to produce a composite material in the form of a plate.

The tensile characteristics and heat conductivity of the plate were measured. Table 2 shows the results. Table 2 shows that the composite materials produced employing the graphite fiber of the present invention have high strength, high modulus and excellent heat conductivity.

**TABLE 1**

| | Sample No. | | | | | |
|---|---|---|---|---|---|---|
| | 1* | 2* | 3** | 4** | 5** | 6** |
| Preoxidation Time (min.) | 48 | 48 | 48 | 55 | 42 | 35 |
| Preoxidized Fiber Density | 1.32 | 1.32 | 1.32 | 1.35 | (1.31) | 1.30 |

| Carbonization Conditions | | | | | | |
|---|---|---|---|---|---|---|
| Temperature (°C) | 1380 | 1380 | 1380 | 1380 | 1380 | 1450 |
| Elongation (%) | 8 | 8 | 1 | 8 | 8 | 8 |

| Properties of Carbon Fiber | | | | | | |
|---|---|---|---|---|---|---|
| Orientation (%) | 82 | 82 | (78) | 81 | 80 | 80 |
| Nitrogen Content (%) | 3.5 | 3.5 | 3.5 | 3.5 | 3.5 | (0.8) |
| Density (g/cm³) | 1.83 | 1.83 | 1.80 | (1.78) | 1.84 | 1.82 |

| Graphitization Conditions | | | | | | |
|---|---|---|---|---|---|---|
| Temperature (°C) | 2880 | 2880 | 2880 | 2880 | 2880 | 2880 |
| Elongation (%) | 7 | 3 | 7 | 6 | 7 | 7 |

| Properties of Graphite Fiber | | | | | | |
|---|---|---|---|---|---|---|
| Tensile Strength(kgf/mm²) | 380 | 355 | (300) | 383 | (283) | (305) |
| Tensile Modulus | | | | | | |
| (x10³ kgf/mm²) | 58.5 | 53.0 | 57.3 | 56.8 | 56.9 | 57.7 |
| Fiber Density (g/cm³) | 1.96 | 1.96 | 1.96 | (1.90) | 1.96 | 1.96 |
| Fiber diameter (»m) | 4.6 | 4.7 | 4.8 | 4.5 | 5.3 | 4.5 |
| Orientation (%) | 93 | 92 | 89 | 91 | 90 | 90 |
| 1) Filament denier of the acrylic fiber used for preparation of Sample 5 was 0.65 2) Values in the parentheses in Tables 1 and 2 are outside the present invention. | | | | | | |

| | | | | | | |
|---|---|---|---|---|---|---|
| Notes: * : Invention | | | | | | |
| **: Comparative | | | | | | |

The following conversions to SI Units apply:

| To convert from | To | Multiply by |
|---|---|---|
| kgf/mm² | GPa | 9.807 x 10⁻³ |
| g/d | cN/tex | 8.826 |
| d | tex | 0.1111 |
| mg/d | cN/tex | 8.826 x 10⁻³ |
| kgf/cm² | MPa | 9.807 x 10⁻² |

## Claims

1. A graphite fiber derived from an acrylic fiber, said graphite fiber having a fiber density of not less than 1.93 g/cm³, a strand tensile strength of not less than 3.43245 GPa (350 kgf/mm²), and a strand tensile modulus of not less than 519.771 GPa (53×10³ kgf/mm²).

2. The graphite fiber as in Claim 1, wherein the graphite fiber has a filament diameter of not more than 7 »m.

3. The graphite fiber as in claim 1, wherein said fiber density is from 1.93 to 2.10 g/cm³.

4. The graphite fiber as in claim 1, wherein said strand tensile strength is from 3.43245 to 5.39385 GPa (350 to 550 kgf/mm²).

5. The graphite fiber as in claim 1, wherein said strand tensile modulus is from 519.771 to 735.525 GPa (53 x 10³ to 75 x 10³ kgf/mm²).

6. The graphite fiber as in claim 1, wherein the filament diameter is from 0.1 to 7 »m.

7. The graphite fiber as in claim 1, wherein the graphite fiber consists of 99.5 to 100% by weight of carbon atoms, less than 0.1% by weight of each of nitrogen atoms, oxygen atoms, and hydrogen atoms, and less than 0.2% by weight of ash.

8. The graphite fiber as in claim 1, wherein the graphite fiber has an orientation of from 85 to 98% at a maximum diffraction at 2ϑ=25.3±0.5°, X-ray diffraction angle, of (002) plane of the graphite crystal.

9. The graphite fiber as in claim 1, wherein the density is from 1.93 to 2.10 g/cm³, the strand tensile strength is from 3.43245 to 5.39385 GPa (350 to 550 kgf/mm²), the strand tensile modulus is from 519.771 to 735.525 GPa (53 x 10³ to 75 x 10³ kgf/mm²), the graphite fiber consists of from 99.5 to 100% by weight of carbon atoms, less than 0.1% by weight of each of nitrogen atoms, oxygen atoms, and hydrogen atoms, and less than 0.2% by weight of ash, and the graphite fiber has an orientation of from 85 to 98% at a maximum diffraction at 2ϑ=25.3±0.5°, X-ray diffraction angle, of (002) plane of the graphite crystal.

10. A method for manufacturing a graphite fiber having a fiber density of not less than 1.93 g/cm³, a strand tensile strength of not less than 3.43245 GPa (350 kgf/mm²), and a strand tensile modulus of not less than 519.771 GPa (53×10³ kgf/mm²), comprising carbonizing a preoxidized fiber derived from an acrylic fiber and having a fiber density of from 1.32 to 1.40 g/cm³ to obtain a carbon fiber having a nitrogen content of not less than 1.0% by weight based on the carbon fiber weight, a fiber density of not less than 1.79 g/cm³ and an orientation of not less than 79% at a maximum diffraction at 2ϑ=25.3±0.5° in X-ray diffraction angle of the (002) plane of the graphite crystal, and graphitizing the thus-obtained carbon fiber in an inert gas at a temperature of not lower than 2,400°C and under a tension to stretch the fiber at least 3% during the graphitization.

11. The method for manufacturing a graphite fiber as in claim 10, wherein the carbon fiber is stretched by 3% to 15% during the graphitization.

12. The method for manufacturing a graphite fiber as in claim 10, wherein the nitrogen content of the carbon fiber is from 1.0 to 8% by weight.

13. The method for manufacturing a graphite fibers as in claim 10, wherein the carbon fiber has an orientation of from 79 to 84% at the maximum diffraction at 2ϑ=25.3±0.5°, X-ray diffraction angle, of (002) plane of the graphite crystal.

14. The method for manufacturing a graphite fiber as in claim 10, wherein the fiber density of the carbon fiber is from 1.79 to 1.85 g/cm³.

15. The method for manufacturing a graphite fiber as in claim 10, wherein the carbon fiber comprises a strand consisting of from 50 to 15,000 filaments.

16. The method for manufacturing a graphite fiber as in claim 10, wherein the acrylic fiber is a polyacrylonitrile fiber or a copolymer fiber composed of not less than 90% by weight of acrylonitrile.

17. The method for manufacturing a graphite fiber as in claim 10, wherein the acrylic fiber has a filament diameter of from 0.1 to 13 »m.

18. The method for manufacturing a graphite fiber as in claim 10, wherein the carbon fiber is derived from an acrylic fiber having a tensile strength of not less than 26.478 cN/tex (3 g/d), a tensile elongation of not less than 5%, and an orientation degree of not less than 88% measured at the X-ray diffraction angle of 2ϑ=17.3 ± 0.3°.

19. The method for manufacturing a graphite fiber as in claim 10, wherein the graphitizing temperature is from 2,400 to 3,300°C.

20. The method for manufacturing a graphite fiber as in claim 18, wherein the carbon fiber is obtained by preoxidizing said acrylic fiber in air at a temperature of from 200 to 350°C under a tension of from 0.617 to 1.765 cN/tex (70 to 200 mg/d) until the fiber density reaches 1.33 to 1.40 g/cm³, and then the thus obtained preoxidized fiber is carbonized in an inert atmosphere at a temperature of from 1,100 to 1,430°C while under a stretching condition so as to result in the orientation degree of from 79% to 84% at the maximum diffraction at 2ϑ=25.3±0.5°, X-ray diffraction angle, of (002) plane of the graphite crystal, until the fiber density becomes least 1.79 to 1.85 g/cm³ and the nitrogen content of from 1.0 to 8% by weight.

21. The method for manufacturing a graphite fiber as in claim 20, wherein carbonizing is conducted under a stretching condition to stretch the fiber in an extent of from 5 to 20%.

## Patentansprüche

1. Von einer Acrylfaser abgeleitete Graphitfaser, wobei die Graphitfaser eine Faserdichte von nicht weniger als 1,93 g/cm³ hat, eine Fadenzugfestigkeit von nicht weniger als 3,43245 GPa (350 kgf/mm²) und einen Fadenzugmodul von nicht weniger als 519,771 GPa (53x10³ kgf/mm²) hat.

2. Graphitfaser gemäß Anspruch 1, bei welcher die Graphitfaser einen Filamentdurchmesser von nicht mehr als 7 »m hat.

3. Graphitfaser gemäß Anspruch 1, bei welcher die Faserdichte 1,93 bis 2,10 g/cm³ beträgt.

4. Graphitfaser gemäß Anspruch 1, bei welcher die Fadenzugfestigkeit von 3,43245 bis 5,39385 GPa (350 bis 550 kgf/mm²) beträgt.

5. Graphitfaser gemäß Anspruch 1, bei welcher die Fadenzugfestigkeit 519,771 bis 735,525 GPa (53 x 10³ bis 75 x 10⁵ kgf/mm²) beträgt.

6. Graphitfaser gemäß Anspruch 1, bei welcher der Filamentdurchmesser 0,1 bis 7 »m beträgt.

7. Graphitfaser gemäß Anspruch 1, bei welcher die Graphitfaser aus 99,5 bis 100 Gew.-% Kohlenstoffatomen, weniger als 0,1 Gew.-% von jeweils Stickstoffatomen, Sauerstoffatomen und Wasserstoffatomen und weniger als 0,2 Gew.-% Asche besteht.

8. Graphitfaser gemäß Anspruch 1, bei welcher die Graphitfaser eine Orientierung von 85 bis 98 % bei einer maximalen Beugung bei 2ϑ = 25,3 ± 0,5°, Röntgenbeugungswinkel der (002) Ebene des Graphitkristalls hat.

9. Graphitfaser gemäß Anspruch 1, in welcher die Dichte 1,93 bis 2,10 g/cm³ beträgt, die Fadenzugfestigkeit 3,43245 bis 5,39385 GPa (350 bis 550 kgf/mm²) ist, der Fadenzugmodul 519,771 bis 735,525 GPa (53 x 10³ bis 75 x 10³ kgf/mm²) ist, die Graphitfaser aus 99,5 bis 100 Gew.-% Kohlenstoffatomen, weniger als 0,1 Gew.-% von jeweils Stickstoffatomen, Sauerstoffatomen und Wasserstoffatomen und weniger als 0,2 Gew.-% Asche besteht, und die Graphitfaser eine Orientierung von 85 bis 98 % bei der Maximalbeugung bei 2ϑ = 25,3 ± 0,5°, Röntgenbeugungswinkel der (002) Ebene des Graphitkristalls hat.

10. Verfahren zur Herstellung einer Graphitfaser mit einer Faserdichte von nicht weniger als 1,93 g/cm³, einer Fadenzugfestigkeit von nicht weniger als 3,43245 GPa (350 kgf/mm²) und einem Fadenzugmodul von nicht weniger als 519,771 GPa (53x10³ kgf/mm²) hat, umfassend das Carbonisieren einer voroxidierten Faser, die sich von einer Acrylfaser ableitet, mit einer Faserdichte von 1,32 bis 1,40 g/cm³ unter Erhalt einer Kohlenstoffaser mit einem Stickstoffgehalt von nicht weniger als 1,0 Gew.-%, bezogen auf das Kohlenfasergewicht, einer Faserdichte von nicht weniger als 1,79 g/cm³ und einer Orientierung von nicht weniger als 79 % bei der Maximalbeugung bei 2ϑ = 25,3 ± 0,5° bei dem Röntgenbeugungswinkel der (002) Ebene des Graphitkristalls, und Graphitisieren der so erhaltenen Kohlenstoffaser in einem Inertgas bei einer Temperatur von nicht niedriger als 2.400°C unter Spannung und Strecken der Faser um wenigstens 3 % während der Graphitisierung.

11. Verfahren zur Herstellung einer Graphitfaser gemäß Anspruch 10, wobei die Kohlenstoffaser während der Graphitisierung um 3 % bis 15 % gestreckt wird.

12. Verfahren zur Herstellung einer Graphitfaser gemäß Anspruch 10, wobei der Stickstoffgehalt der Kohlenstoffaser 1,0 bis 8 Gew.-% beträgt.

13. Verfahren zur Herstellung einer Graphitfaser gemäß Anspruch 10, wobei die Kohlenstoffaser eine Orientierung von 79 bis 84 % bei der Maximalbeugung bei 2ϑ = 25,3 ± 0,5°, Röntgenbeugungswinkel der (002) Ebene des Graphitkristalls hat.

14. Verfahren zur Herstellung einer Graphitfaser gemäß Anspruch 10, wobei die Faserdichte der Kohlenstoffaser 1,79 bis 1,85 g/cm³ beträgt.

15. Verfahren zur Herstellung einer Graphitfaser gemäß Anspruch 10, wobei die Kohlenstoffaser einen Faden, bestehend aus 50 bis 15.000 Filamenten umfaßt.

16. Verfahren zur Herstellung einer Graphitfaser gemäß Anspruch 10, wobei die Acrylfaser eine Polyacrylnitrilfaser oder eine Copolymerfaser, die sich aus nicht weniger als 90 Gew.-% an Acrylnitril zusammensetzt, ist.

17. Verfahren zur Herstellung einer Graphitfaser gemäß Anspruch 10, bei dem die Acrylfaser einen Filamentdurchmesser von 0,1 bis 13 »m hat.

18. Verfahren zur Herstellung einer Graphitfaser gemäß Anspruch 10, wobei die Kohlenstoffaser sich von einer Acrylfaser mit einer Zugfestigkeit von nicht weniger als 26,478 cN/tex (3 g/d) einer Zugdehnung von nicht weniger als 5 % und einem Orientierungsgrad von nicht weniger als 88 %, bezogen bei dem Röntgenbeugungswinkel von 2ϑ = 17,3 ± 0,3° hat.

19. Verfahren zur Herstellung einer Graphitfaser gemäß Anspruch 10, wobei die Graphitisierungstemperatur 2.400 bis 3.300°C beträgt.

20. Verfahren zur Hertellung einer Graphitfaser gemäß Anspruch 18, bei dem die Kohlenstoffaser erhalten wurde durch Voroxidieren der Acrylfaser an der Luft bei einer Temperatur von 100 bis 350°C unter einer Spannung von 0,617 bis 1,765 cN/tex (70 bis 200 mg/d) bis die Faserdichte 1,33 bis 1,40 g/cm³ erreicht, worauf man dann die erhaltene voroxidierte Faser in einer Inertatmosphäre bei einer Temperatur von 1.100 bis 1.430°C unter Streckbedingungen carbonisiert, so daß man einen Orientierungsgrad von 79 % bis 84 % bei der Maximalbeugung bei 2ϑ = 25,3 ± 0,5°, Röntgenbeugungswinkel der (002) Ebene des Graphitkristalls erhält, bis die Faserdichte wenigstens 1,79 bis 1,85 g/cm³ beträgt, und der Stickstoffgehalt 1,0 bis 8 Gew.-% ist.

21. Verfahren zur Herstellung einer Graphitfaser gemäß Anspruch 20, bei dem man das Carbonisieren unter Streckbedingungen durchführt und die Faser bis zu einem Ausmaß von 5 bis 20 % streckt.

## Revendications

1. Fibre de graphite obtenue à partir d'une fibre acrylique, ladite fibre de graphite ayant une densité de fibre non inférieure à 1,93 g/cm³, une résistance à la traction du brin non inférieure à 3,43245 GPa (350 kgf/mm²) et un module de traction du brin non inférieur à 519,771 GPa (53x10³ kgf/mm²).

2. Fibre de graphite selon la revendication 1, dans laquelle la fibre de graphite a un diamètre des filaments non supérieur à 7 »m.

3. Fibre de graphite selon la revendication 1, dans laquelle la densité de ladite fibre est de 1,93 à 2,10 g/cm³.

4. Fibre de graphite selon la revendication 1, dans laquelle ladite résistance à la traction du brin est de 3,43245 à 5,39385 GPa (350 à 550 kgf/mm²).

5. Fibre de graphite selon la revendication 1, dans laquelle le module de traction du brin est de 519,771 à 735,525 GPa (53 x 10³ à 75 x 10³ kgf/mm²).

6. Fibre de graphite selon la revendication 1, dans laquelle le diamètre des filaments est de 0,1 à 7 »m.

7. Fibre de graphite selon la revendication 1, dans laquelle la fibre de graphite est constituée à 99,5 à 100 % en poids par des atomes de carbone, à moins de 0,1 % en poids par chacun des atomes d'azote, des atomes d'oxygène et des atomes d'hydrogène, et à moins de 0,2 % en poids par de la cendre.

8. Fibre de graphite selon la revendication 1, dans laquelle la fibre de graphite a une orientation de 85 à 98 % à une diffraction maximale à un angle de diffraction des rayons X 2ϑ = 25,3 ± 0,5°, du plan (002) du cristal de graphite.

9. Fibre de graphite selon la revendication 1, dans laquelle la densité est de 1,93 à 2,10 g/cm³, la résistance à la traction du brin est de 3,43245 à 5,39385 GPa (350 à 550 kgf/mm²), le module de traction du brin est de 519,771 à 735,525 GPa (53 x 10³ à 75 x 10³ kgf/mm²), la fibre de graphite est constituée à 99,5 à 100 % en poids par des atomes de carbone, à moins de 0,1 % en poids par chacun des atomes d'azote, des atomes d'oxygène et des atomes d'hydrogène, et à moins de 0,2 % en poids par de la cendre, et la fibre de graphite a une orientation de 85 à 98 % à une diffraction maximale à un angle de diffraction des rayons X 2ϑ = 25,3 ± 0,5°, du plan (002) du cristal de graphite.

10. Procédé pour fabriquer une fibre de graphite ayant une densité de fibre non inférieure à 1,93 g/cm³, une résistance à la traction du brin non inférieure à 3,43245 GPa (350 kgf/mm²) et un module de traction du brin non inférieur à 519,771 GPa (53 x 10³ kgf/mm²), comprenant la carbonisation d'une fibre préoxydée obtenue à partir d'une fibre acrylique et ayant une densité de fibre de 1,32 à 1,40 g/cm³, pour obtenir une fibre de carbone ayant une teneur en azote non inférieure à 1,0 % en poids sur la base du poids de la fibre de carbone, une densité de fibre non inférieure à 1,79 g/cm³ et une orientation non inférieure à 79 % à une diffraction maximale à dans un angle de diffraction des rayons X 2ϑ = 25,3 ± 0,5°, du plan (002) du cristal de graphite, et la graphitisation de la fibre de carbone ainsi obtenue dans un gaz inerte, à une température non inférieure à 2 400 °C et sous une tension pour étirer la fibre d'au moins 3 % durant la graphitisation.

11. Procédé pour fabriquer une fibre de graphite selon la revendication 10, dans lequel la fibre de carbone est étirée de 3 % à 15 % durant la graphitisation.

12. Procédé pour fabriquer une fibre de graphite selon la revendication 10, dans lequel la teneur en azote de la fibre de carbone est de 1,0 à 8 % en poids.

13. Procédé pour fabriquer des fibres de carbone selon la revendication 10, dans lequel la fibre de carbone a une orientation de 79 à 84 % à la diffraction maximale dans l'angle de diffraction des rayons X 2ϑ = 25,3 ± 0,5° du plan (002) du cristal de graphite.

14. Procédé pour fabriquer une fibre de graphite selon la revendication 10, dans lequel la densité de fibre de la fibre de carbone est de 1,79 à 1,85 g/cm³.

15. Procédé pour fabriquer une fibre de graphite selon la revendication 10, dans lequel la fibre de carbone comprend un brin constitué de 50 à 15 000 filaments.

16. Procédé pour fabriquer une fibre de graphite selon la revendication 10, dans lequel la fibre acrylique est une fibre de polyacrylonitrile ou une fibre de copolymère composée de pas moins de 90 % en poids d'acrylonitrile.

17. Procédé pour fabriquer une fibre de graphite selon la revendication 10, dans lequel la fibre acrylique a un diamètre des filaments de 0,1 à 13 »m.

18. Procédé pour fabriquer une fibre de graphite selon la revendication 10, dans lequel la fibre de carbone est obtenue à partir d'une fibre acrylique ayant une résistance à la traction non inférieure à 26,478 cN/tex (3 g/d), un allongement à la traction non inférieur à 5 % et un degré d'orientation non inférieur à 88 % mesuré à l'angle de diffraction des rayons X de 2ϑ = 17,3 ± 0,3°.

19. Procédé pour fabriquer une fibre de graphite selon la revendication 10, dans lequel la température de graphitisation est de 2 400 à 3 300 °C.

20. Procédé pour fabriquer une fibre de graphite selon la revendication 18, dans lequel la fibre de carbone est obtenue en préoxydant ladite fibre acrylique dans l'air à une température de 200 à 350 °C, sous une tension de 0,617 à 1,765 cN/tex (70 à 200 mg/d) jusqu'à ce que la densité de la fibre atteigne 1,33 à 1,40 g/cm³, puis la fibre préoxydée ainsi obtenue est carbonisée dans une atmosphère inerte à une température de 1 100 à 1 430 °C tout en étant dans une condition d'étirement de façon à obtenir le degré d'orientation de 79 % à 84 % à la diffraction maximale à l'angle de diffraction des rayons X 2ϑ = 25,3 ± 0,5° du plan (002) du cristal de graphite, jusqu'à ce que la densité de la fibre devienne au moins 1,79 à 1,85 g/cm³ et la teneur en azote de 1,0 à 8 % en poids.

21. Procédé pour fabriquer une fibre de graphite selon la revendication 20, dans lequel la carbonisation est effectuée dans une condition d'étirement pour étirer la fibre dans une mesure de 5 à 20 %.
